

## UNITED STATES PATENT OFFICE.

JUDSON A. DE CEW, OF MOUNT VERNON, NEW YORK, ASSIGNOR TO PROCESS ENGINEERS INC., OF NEW YORK, N. Y.

## METHOD OF HYDRATING CELLULOSE FIBERS.

No Drawing.

Application filed June 7, 1924. Serial No. 718,656.

To all whom it may concern:

Be it known that JUDSON A. DE CEW, a citizen of the United States, residing at Mount Vernon, in the county of Westchester and State of New York, has invented certain new and useful Improvements in Methods of Hydrating Cellulose Fibers, of which the following is a specification.

In the art of paper making the cellulose fibers from which the paper or board is made are mixed and treated in machines called beating engines where the fibers are prepared by treating them between the knives of the revolving roll and the knives of the fixed bedplate.

The action which takes place under these conditions may be a cutting action which shortens the fibers or it may be a different action, depending on the method of operation which results in the wetting of the fibers, by the squeezing and beating action they receive between the revolving roll and the bedplate. For some classes of papers, it is desirable to wet the fibers very thoroughly so that they are softened and swollen and become very pliable and this action is generally called hydration.

The common practice in treating these fibers in the beating engine is to carry on the coloring and sizing reactions that are to be produced at the same time as the hydration of the fibers takes place, the size and alum being used for sizing being added before the beater is discharged.

This means that much of the hydration of the beater is carried on while the stock is in an acid condition, for the sizing of paper always requires an excess of sulphate of alumina which has an acid reaction.

For some classes of papers a large percent of the hydration is produced in the beating engine while for other kinds of paper, such as kraft paper or rag and sulphite papers, a large part and sometimes all of the hydration is produced in another machine known as a Jordan engine.

The Jordan engine is also a machine with revolving knives beating against fixed knives and this machine being standard equipment in nearly every paper mill, is always operated on stock which has been previously made acid with sulphate of alumina, while in the beating engine.

The Jordan engine is a machine which re-

quires a large amount of power to operate, 55 requiring from 150 to 400 horsepower for each machine, depending upon the character of the paper pulp being treated.

In the manufacture of kraft which is a common variety of wrapping paper, the 60 Jordan engine is relied upon by many mills to produce nearly all of the hydration that takes place.

Any process effecting the efficiency of this piece of equipment has an important bearing upon the quality of the finished product.

I have discovered after making both laboratory and mill tests that a different kind of hydration takes place in fibers that are beaten while in an alkaline or neutral 70 condition than those that are being hydrated while in an acid condition in the presence of sulphate of alumina.

I have discovered that the hydration is most rapid while the stock is in an alkaline 75 condition and that the hydration is the slowest when it takes place in the presence of a solution of sulphate of alumina which makes the fibers astringent, stiff and prevents them from absorbing the water of hydration and 80 also makes the fibers more easily cut by the knives of the beating engine or the Jordan.

In order to produce rapid hydration with the minimum of power and in order to produce the best quality of paper, I beat the 85 stock while in a neutral or alkaline condition and discharge it from the beating engine without adding sulphate of alumina to produce an acid condition.

The fibers are then treated in the Jordan 90 while still in a neutral or alkaline condition where it undergoes further degrees of hydration and refinement and after this action is completed and the stock is ready for the paper machine, it is then mixed with sulphate of alumina to produce the acid condition necessary for sizing, after which it is passed to the screens or the paper machine.

The effect of this process is to produce a fiber which is slightly alkaline in its interior 100 and slightly acid on its outer surface. Such a fiber has special paper making properties that are of particular value in the production of a strong and pliable paper.

By this process I have obtained certain 105 distinct advantages from those now being obtained by methods in common use. The advantages are as follows: (1) The hydrat-

ing action in the Jordan is much more efficient and less power is used by the Jordan to produce the same result; (2) the paper produced by this method of beating in the 5 Jordan is stronger and more pliable; (3) there is no corrosion of the knives in the beating engine or Jordan; (4) sulphate of alumina is not in contact with the fibers long enough to make them astringent, although it will react completely with the 10 rosin size within the time allowed.

I, therefore, claim as my invention:

15 1. A method of hydrating cellulose fibers, which consists in beating them in both beater and Jordan while in an alkaline condition.

2. A method of hydrating cellulose fibers, which consists in passing them through a

Jordan engine while in an alkaline condition.

20

3. A method of treating cellulose fibers for paper making, which consists in hydrating the fibers by beating and jordaning them in the presence of a soluble alkali until the fibers are made pliable by the penetration of the alkali, and then neutralizing the alkali that is on the surface of the fibers and in the solution surrounding the fibers, by means 25 of sulphate of alumina.

4. A pliable paper product made from 30 cellulose fibers, having the interior of each fiber slightly alkaline and the surface of each fiber slightly acid.

In testimony whereof I affix my signature.

JUDSON A. DE CEW.